

## UNITED STATES PATENT OFFICE

CAMPBELL R. McCULLOUGH AND RUSSELL L. JENKINS, OF ANNISTON, ALABAMA, ASSIGNORS, BY MESNE ASSIGNMENTS, TO SWANN RESEARCH, INC., OF BIRMINGHAM, ALABAMA, A CORPORATION OF ALABAMA

## TRANSFORMER OIL

No Drawing.

Application filed October 28, 1929. Serial No. 403,116.

This invention relates to a new insulating di-electric liquid and particularly to a liquid in which electrical conductors may be immersed. It is particularly adapted to be used as a filling material for oil immersed

transformers. At present, mineral oils are used to fill transformers, which oils, however, are objectionable in that they tend to form sludges which must be removed by filtration from time to time. Furthermore, they have a relatively low flash point, which makes the product something of a fire hazard.

Another product which has been proposed is a mixture of diphenyl oxide and carbon tetrachloride. This material, however, has a relatively high freezing point and consequently is disadvantageous when used in cold weather.

We have found that several of the lower chlorinated diphenyls can be used advantageously and the above difficulties largely overcome. For example, we have found that when a mixture is made containing approximately 75% of 2-chlorodiphenyl (ortho) and 25% 4-chlorodiphenyl (para), a eutectic mixture is obtained which has a freezing point at 14° C. It has a flash point at 127° to 129° C., and a fire point at 200° C.

The freezing point of the above mixture may be lowered to a point considerably below 0° C. in the following manner:—Take 55% of the above mixture of chloro-diphenyls and mix it with 45% of a product obtained in the following manner:

Chlorinate diphenyl, using iron as a catalyst, until it reaches a specific gravity of 1.379 at 20° C. This corresponds to a chlorine content in the neighborhood of 42% by weight. The product is washed with dilute hydrochloric acid, then with water, and finally with soda ash to neutralize acidity, and dried. The entire charge is then distilled at atmospheric pressure, no attempt being made to separate any fraction.

On mixing the product with the mixture given above it will be found to have the following properties:

|                      |                                |    |
|----------------------|--------------------------------|----|
| Density              | 1. 246 at 25° C.               |    |
| Viscosity            | 45 seconds Saybolt at 37.8° C. | 50 |
| Solidifies           | minus 30° C.                   |    |
| Flash point (5 sec.) | 140° C.                        |    |
| Flame point          | 218° C.                        |    |

The density of the oil may vary somewhat depending upon how far the chlorination is carried, for example it may vary between 1.22 and 1.28 at 25° C. A higher chlorine content will also increase the viscosity which we have found to vary between 40–50 seconds at 37.8° C.

While the proportions given above will give a satisfactory oil of the properties shown above, it should be realized that other proportions are possible and may be desirable for certain particular uses.

## What we claim is:

1. A dielectric comprising a liquid mixture of chlorinated diphenyl having a solidification point below 14° C. 65

2. A dielectric comprising a mixture of ortho- and para-chlorodiphenyl, having a solidification point in the neighborhood below 14° C. and a flash point above 127° C. 70

3. A dielectric comprising a mixture of ortho- and para-chlorodiphenyl in the eutectic proportions. 75

4. A dielectric comprising a liquid mixture of ortho- and para- with a higher chlorinated diphenyl, said liquid mixture having a solidification point in the neighborhood of minus 30° C. 80

5. A dielectric comprising a liquid mixture of 55% of the eutectic mixture of ortho- and para-chlorodiphenyl with 45% of an oil formed by chlorinating diphenyl to a specific gravity of 1.379 at 20° C. 85

6. A dielectric comprising a distilled substance of substantially 41.25% ortho-chlorodiphenyl, 13.75% para-chlorophenyl and 45% of a product formed by chlorinating 90

diphenyl to a density in the neighborhood of 1.379 at 20° C.

7. A dielectric comprised of chlorinated diphenyl having a density between 1.22 and 1.28.

8. A dielectric comprised of chlorinated diphenyl, having a density in the neighborhood of 1.25 and a flash point in the neighborhood of 140° C.

10. 9. A dielectric comprising a liquid chlorinated diphenyl.

In testimony whereof we affix our signatures.

15 CAMPBELL R. McCULLOUGH.  
RUSSELL L. JENKINS.

20

25

30

35

40

45

50

55

60

65